

## UNITED STATES PATENT OFFICE

2,226,103

## PROCESS FOR MICA FLOTATION

Francis X. Tartaron and Leslie Roth Harrison, Jr.,  
Mulberry, Fla., assignors to Phosphate Recovery  
Corporation, New York, N. Y., a corporation of  
Delaware

No Drawing. Application September 23, 1939,  
Serial No. 296,224

6 Claims. (Cl. 209—166)

This invention relates to a process for separating mica from mixtures containing mica and impurities such as feldspar, quartz, and clay, for example, by means of froth flotation. In carrying out this invention a reagent is used which when mixed with the ore pulp causes accumulation of the mica selectively in the froth.

The invention has been tried extensively with ore from Sprucepine, North Carolina. The mica occurs in this ore as muscovite and is intermixed with feldspar, quartz, and clay. Different fractions of the material in particles of various sizes have been successfully treated by this process.

In carrying out the present invention, successful commercial concentration of the mica in the ore is obtained by the use of alkali resinate as the flotation collector. Although the addition of a frothing agent is not essential to the process, certain frothers, such as pine oil and P. T. 101, for example, have been found to assist in the flotation. The flotation collector, alkali resinate, is added to a dilute pulp having therein about 10-20% solids in a flotation machine, the pulp is agitated for a short period of time to mix the contents of the flotation machine, then the flotation operation is consummated. The mica concentrate collects in the upper portion of the flotation machine and is skimmed off of the surface of the pulp. It has been found to be desirable to repulp with water in some instances and refloat so as to further purify the desired product.

A mica product or concentrate weighing less than 20 lbs. per cubic foot, which is considered highly desirable in the trade, can be readily and rapidly produced by this process.

The following examples illustrate the process of this invention. However, the invention is not limited to these examples, as considerable variation can be made without departing from the spirit or scope of the invention.

## Example No. 1

The material that was treated was a "fine sand" product from the washer of Kaolin, Inc., Sprucepine, North Carolina. It contained about 2% of particles plus 48-mesh and 60% minus 100-mesh. The mica was about 20% of the material treated and consisted of muscovite. Impurities were feldspar, quartz, and clay.

To a pulp of this material containing about 10% solids in a M. S. laboratory flotation machine, the reagents mentioned below were added, followed by the agitation period also stated. The pulp was then frothed and the concentrate was collected. This froth concentrate was repulped

and more reagent was added. A second flotation was consummated, giving the finished product. Rejects of first flotation are tailings to be discarded. Rejects of second flotation are middlings to be returned to the flotation circuit and further values recovered therefrom.

|                      | Rougher float     | Cleaner float | 10   |
|----------------------|-------------------|---------------|------|
| Sodium resinate..... | lbs. per ton..... | 3.00          | 1.40 |
| Pine oil.....        | do.....           | 0.42          | —    |
| Mixing time.....     | seconds.....      | 15            | 15   |
| Time of float.....   | minutes.....      | 3             | 1½   |

| Product   | Percent weight | Pounds per cubic foot | 15 |
|-----------|----------------|-----------------------|----|
| Feed..... | 100.0          | 41.3                  |    |
| Conc..... | 18.8           | 19.5                  |    |
| Midd..... | 13.8           | —                     | 20 |
| Tail..... | 67.4           | —                     |    |

## Example No. 2

The material treated was "sand box settling" of washer of Kaolin, Inc. This product had the same size distribution of particles as in Example 1, but contained 33% mica as muscovite with impurities of feldspar, quartz, and clay.

The method of treatment was identical with that given in Example No. 1.

|                      | Rougher float     | Cleaner float | 35   |
|----------------------|-------------------|---------------|------|
| Sodium resinate..... | lbs. per ton..... | 3.00          | 1.40 |
| Pine oil.....        | do.....           | 0.42          | 0    |
| Mixing time.....     | seconds.....      | 15            | 15   |
| Flotation time.....  | minutes.....      | 3             | 2½   |

| Product   | Percent weight | Pounds per cubic foot | 40 |
|-----------|----------------|-----------------------|----|
| Feed..... | 100.0          | 32.8                  |    |
| Conc..... | 32.4           | 15.5                  |    |
| Midd..... | 18.6           | —                     | 45 |
| Tail..... | 49.3           | —                     |    |

## Example No. 3

The mica-containing product was scalped from 50- and 60-mesh screens at the plant of Kaolin, Inc. This material contained 85% of mica as muscovite, impurities being feldspar, quartz, and clay. The sizes ranged from 20- to 60-mesh, and the cubic weight was 20 lbs. per

cubic foot. To the ore pulped with water so as to contain 10% solids, reagents were added as shown below in five tests illustrating the effect of increasing quantities of the resinate. The pulp was agitated 15 seconds. Flotation was then carried out. The froth was not retreated.

| 10 | Reagents,<br>pounds per<br>ton |             | Froth product     |                             |
|----|--------------------------------|-------------|-------------------|-----------------------------|
|    | Sodium<br>resinate             | Pine<br>oil | Percent<br>weight | Pounds<br>per cubic<br>foot |
| 15 | 3.00                           | 0.42        | 56.2              | 15.2                        |
|    | 5.00                           | 0.42        | 62.0              | 14.8                        |
|    | 7.00                           | 0.42        | 69.0              | 15.6                        |
|    | 10.00                          | 0.42        | 72.4              | 15.8                        |
|    | 15.00                          | 0.42        | 73.8              | 15.5                        |

**20** *Example No. 4*

The procedure is the same as in Example 1, except that a second cleaning operation is used.

| 25                       | Reagents and conditions | Rougher float | Cleaner float | Recleaner float |
|--------------------------|-------------------------|---------------|---------------|-----------------|
| Sodium resinate          | lbs. per ton            | 3.00          | 1.40          | 0.80            |
| P. T. 101 as the frother | do                      | 0.42          |               |                 |
| Mixing time              | seconds                 | .15           | 15            | 15              |
| 30 Flotation time        | minutes                 | 1½            | 1½            | 1½              |

| Product      | Percent weight | Cubic weight (pounds per cubic foot) |
|--------------|----------------|--------------------------------------|
| Feed.....    | 100.0          | 41.3                                 |
| Cond.....    | 8.9            | 19.8                                 |
| Midd.-2..... | 4.2            |                                      |
| Midd.-1..... | 15.9           |                                      |
| Tail.....    | 71.0           |                                      |

**Example No. 5**

The procedure is the same as in Example 4.

| Reagents and conditions           | Rougher float   | Cleaner float   | Recleaner float |
|-----------------------------------|-----------------|-----------------|-----------------|
| Sodium resinate..... lbs. per ton | 3.00            | 1.40            | 0.80            |
| Cresol as the frother..... do     | 0.41            |                 |                 |
| Mixing time..... seconds          | 15              | 15              | 15              |
| Flotation time..... minutes       | 1 $\frac{1}{2}$ | 1 $\frac{1}{2}$ | 1 $\frac{1}{2}$ |

| Product | Percent weight | Cubic weight (pounds per cubic foot) |
|---------|----------------|--------------------------------------|
| Feed    | 100.0          | 41.3                                 |
| Cond.   | 10.9           | 19.9                                 |
| Midd.—2 | 4.8            |                                      |
| Midd.—1 | 15.2           |                                      |
| Tall    | 60.1           |                                      |

**What is claimed is:**

1. The process of concentrating mica by froth flotation, which comprises pulping the ore with water, mixing therein alkali resinate, and subjecting the pulp to a froth flotation treatment. 25
  2. The process according to claim 1, in which the resinate is sodium resinate.
  3. The process according to claim 1, in which there are two flotation treatments and a part of the resinate is added to first treatment and a part to second treatment. 30
  4. The process according to claim 1, in which a frother is used.
  5. The process according to claim 1, in which pine oil is added as a frother. 35
  6. The process according to claim 1, in which the pulp has therein about ten percent to twenty percent solids.

## FRANCIS X. TARTARON.

LESLIE ROTH HARRISON, JR.